

3,218,155

## METHOD OF OPERATING METALLURGICAL FURNACES

Julius H. Strassburger, Coraopolis, Pa., assignor to National Steel Corporation, a corporation of Delaware  
No Drawing. Filed Dec. 22, 1960, Ser. No. 77,507  
23 Claims. (Cl. 75—42)

This application is a continuation-in-part of Serial No. 54,366, filed September 7, 1960, and now abandoned.

This invention relates to blast furnaces and more particularly to improvements in the method of operating blast furnaces.

Conventional blast furnaces comprise a hearth, a stack and bosh between the hearth and the stack. The blast, comprising essentially compressed air, is blown through tuyeres mounted in the bosh into the upper portion of the hearth, and the burden, including specific proportions of limestone, ferrous bearing material and carbonaceous material is charged into the furnace at the top of the stack. The ferrous bearing material is usually iron ore and may include some scrap metal, sinter or other material and the carbonaceous material is usually coke. The charge moves down the shaft of the furnace and when it reaches a zone adjacent the tuyeres the coke is burned by the incoming blast to melt the iron ore producing molten pig iron and the hot gaseous products of combustion flow up through the stack, preheating the descending charge and reducing the iron ore as it approaches the combustion zone, and out through the top of the furnace.

The quantity and physical character of material discharged into the top of the furnace as burden and the volume of blast gas blown into the furnace are calculated and controlled to maintain the highest possible rate of pig iron production with minimum coke consumption and with minimum flue dust production. The volume of blast gas required depends upon the physical characteristics of the furnace and the components of the burden and must be carefully controlled in order to maintain a smooth operating furnace. It is known that an insufficient volume of blast gas results in low pig iron production and high coke rates, while excessive blast gas increases flue dust production without a corresponding rise in iron production.

The driving rate of a blast furnace is a measure of the quantity of carbon gasified at the tuyeres by combustion of coke. Since coke combustion is influenced by the oxygen available and by the existing temperature it has been proposed in the past to increase the production of blast furnaces without substantially increasing the volume of blast gas by either enriching the blast gas with oxygen or by blowing the blast gas to the furnace at an elevated temperature. It was found however that the mere enrichment of the blast gas with oxygen or the mere increase in temperature of the blast gas did not produce the expected results as the furnace either ran cold due to resulting high velocity of upwardly flowing bosh gas or that the movement of the burden slowed down and became intermittent or at times actually stopped and caused the furnace to hang which was followed by violent slips. It was theorized that the inability to obtain a smooth operating furnace when enriching the blast gas with oxygen or by elevating the temperature of the blast gas results from the fact that oxygen enrichment of the blast gas or increase in blast gas temperature produces more intensified burning of the coke and thereby shortens the combustion zones in front of the tuyeres, and that reducing the size of the combustion zones enlarges the mass of burden centrally positioned with respect to the hearth and decreases the area available for upward flow of combustion gases. It was then discovered that the addition of moisture to the blast gas made it possible to

obtain a smooth operating furnace when enriching the blast gas with oxygen or when blowing the blast gas at an elevated temperature. The addition of moisture or its equivalent to blast gas makes it possible to enrich the blast gas with oxygen or to blow the blast gas at a higher temperature and thereby improve furnace production. While added moisture comprises a cheap source of oxygen which is introduced into the furnace without nitrogen and also provides a source of hydrogen gas which is more efficient than carbon monoxide in reducing iron ore, higher rates of iron production would be obtained if it were possible to reduce the quantity of moisture required since disassociation of water is an endothermic reaction absorbing heat from the combustion zone and since the coke rate is proportional to the temperature.

It is well known that blast furnaces may be operated to produce, within limits, products of specified characteristics and it is desirable to obtain smooth operations in blast furnaces producing pig iron of different chemical compositions, temperatures, etc. Accordingly, the obtaining of a smooth operating furnace by means of moisture additions to the blast gas includes the feature of controlling the characteristics of the product by such moisture additions.

It is, therefore, a principal object of the present invention to provide a novel method of operating a blast furnace by which maximum iron production is obtained with a minimum coke rate.

Another object is to provide a novel method of operating a blast furnace by which combustion of coke is intensified without correspondingly increasing the volume of blast gas in such a manner as to require minimum moisture additions to the blast gas.

It has been established that predetermined quantities of moisture are required to be added to oxygen enriched blast gas or to blast gas at an elevated temperature in order to obtain smooth operating furnaces. The quantity of moisture required may be considered as depending for the most part upon the percentage of oxygen enrichment or upon the blast temperature although the moisture actually required may be influenced by the physical characteristics of the furnace or by the constituents of the burden. In particular, the quantity of moisture required in blast gas at about 1100° F. for varying percentages of oxygen enrichment is shown in Table I.

TABLE I

| Oxygen enrichment (percent): | Moisture in blast (grains per cubic foot) |
|------------------------------|-------------------------------------------|
| 1.0                          | 3 to 7                                    |
| 1.5                          | 4 to 8                                    |
| 2.0                          | 5 to 10                                   |
| 2.5                          | 7 to 13                                   |
| 3.0                          | 9 to 16                                   |
| 3.5                          | 11 to 19                                  |
| 4.0                          | 13 to 22                                  |
| 4.5                          | 15 to 25                                  |
| 5.0                          | 17 to 28                                  |

It has also been established that under average conditions about 2.5 to 3.5 grains of moisture per cubic foot of blast gas is required to maintain a smooth operating furnace when blown with blast gas at a temperature of about 1100° F. without oxygen enrichment, and that about 1 grain of moisture per cubic foot of blast gas is required to be added to the blast gas upon each 30° F. increase of the blast gas temperature. From the foregoing, it is possible to ascertain the quantity of moisture that would be expected to be necessary in blast gas at varying temperatures and at various percentages of oxygen enrichment in order to obtain a smooth operating furnace. Tables II through XI disclose the range of moisture required throughout a blast temperature range

of 1100° F. to 2500° F. for oxygen enrichment percentages from 0 to 10.

TABLE II.—0% OXYGEN ENRICHMENT

| Blast Temperature, °F. | Moisture expected to be required (grains per cubic foot) | Moisture required according to present invention (grains per cubic foot) |
|------------------------|----------------------------------------------------------|--------------------------------------------------------------------------|
| 1,100                  | 2.5 to 3.5                                               | 2.5 to 3.5                                                               |
| 1,200                  | 5.8 to 6.8                                               | 5.8 to 6.8                                                               |
| 1,300                  | 9.1 to 10.1                                              | 9.1 to 10.1                                                              |
| 1,400                  | 12.4 to 13.4                                             | 8.4 to 9.4                                                               |
| 1,500                  | 15.7 to 16.7                                             | 11.7 to 12.7                                                             |
| 1,600                  | 19.0 to 20.0                                             | 15.0 to 16.0                                                             |
| 1,700                  | 22.3 to 23.3                                             | 18.3 to 19.3                                                             |
| 1,800                  | 25.6 to 26.6                                             | 21.6 to 22.6                                                             |
| 1,900                  | 28.9 to 29.9                                             | 24.9 to 25.9                                                             |
| 2,000                  | 32.2 to 33.2                                             | 28.2 to 29.2                                                             |
| 2,100                  | 35.5 to 36.5                                             | 31.5 to 32.5                                                             |
| 2,200                  | 38.8 to 39.8                                             | 34.8 to 35.8                                                             |
| 2,300                  | 42.1 to 43.1                                             | 38.1 to 39.1                                                             |
| 2,400                  | 45.4 to 46.4                                             | 41.4 to 42.4                                                             |
| 2,500                  | 48.7 to 49.7                                             | 44.7 to 45.7                                                             |

5

TABLE VI.—2.5% OXYGEN ENRICHMENT

| Blast Temperature, °F. | Moisture expected to be required (grains per cubic foot) | Moisture required according to present invention (grains per cubic foot) |
|------------------------|----------------------------------------------------------|--------------------------------------------------------------------------|
| 1,100                  | 7 to 13                                                  | 7 to 13                                                                  |
| 1,200                  | 10.3 to 16.3                                             | 10.3 to 18.3                                                             |
| 1,300                  | 13.6 to 19.6                                             | 13.6 to 19.6                                                             |
| 1,400                  | 16.9 to 22.9                                             | 16.9 to 22.9                                                             |
| 1,500                  | 20.2 to 26.2                                             | 16.2 to 22.2                                                             |
| 1,600                  | 23.5 to 29.5                                             | 19.5 to 25.5                                                             |
| 1,700                  | 26.8 to 32.8                                             | 22.8 to 28.8                                                             |
| 1,800                  | 30.1 to 36.1                                             | 26.1 to 32.1                                                             |
| 1,900                  | 33.4 to 39.4                                             | 29.4 to 35.4                                                             |
| 2,000                  | 36.7 to 42.7                                             | 32.7 to 38.7                                                             |
| 2,100                  | 40.0 to 46.0                                             | 36.0 to 42.0                                                             |
| 2,200                  | 43.3 to 49.3                                             | 39.3 to 45.3                                                             |
| 2,300                  | 46.6 to 52.6                                             | 42.6 to 48.6                                                             |
| 2,400                  | 49.9 to 55.9                                             | 45.9 to 51.9                                                             |
| 2,500                  | 53.2 to 59.2                                             | 49.2 to 55.2                                                             |

20

TABLE VII.—3.0% OXYGEN ENRICHMENT

| Blast Temperature, °F. | Moisture expected to be required (grains per cubic foot) | Moisture required according to present invention (grains per cubic foot) |
|------------------------|----------------------------------------------------------|--------------------------------------------------------------------------|
| 1,100                  | 3 to 7                                                   | 3 to 7                                                                   |
| 1,200                  | 6.3 to 10.3                                              | 6.3 to 10.3                                                              |
| 1,300                  | 9.6 to 13.6                                              | 9.6 to 13.6                                                              |
| 1,400                  | 12.9 to 16.9                                             | 12.9 to 16.9                                                             |
| 1,500                  | 16.2 to 20.2                                             | 12.2 to 16.2                                                             |
| 1,600                  | 19.5 to 23.5                                             | 15.5 to 19.5                                                             |
| 1,700                  | 22.8 to 26.8                                             | 18.8 to 22.8                                                             |
| 1,800                  | 26.1 to 30.1                                             | 22.1 to 26.1                                                             |
| 1,900                  | 29.4 to 33.4                                             | 25.4 to 29.4                                                             |
| 2,000                  | 32.7 to 36.7                                             | 28.7 to 32.7                                                             |
| 2,100                  | 36.0 to 40.0                                             | 32.0 to 36.0                                                             |
| 2,200                  | 39.3 to 43.3                                             | 35.3 to 39.3                                                             |
| 2,300                  | 42.6 to 46.6                                             | 38.6 to 42.6                                                             |
| 2,400                  | 45.9 to 49.9                                             | 41.9 to 45.9                                                             |
| 2,500                  | 49.2 to 53.2                                             | 45.2 to 49.2                                                             |

25

| Blast Temperature, °F. | Moisture expected to be required (grains per cubic foot) | Moisture required according to present invention (grains per cubic foot) |
|------------------------|----------------------------------------------------------|--------------------------------------------------------------------------|
| 1,100                  | 9 to 16                                                  | 9 to 16                                                                  |
| 1,200                  | 12.3 to 19.3                                             | 12.3 to 19.3                                                             |
| 1,300                  | 15.6 to 22.6                                             | 15.6 to 22.6                                                             |
| 1,400                  | 18.9 to 25.9                                             | 18.9 to 25.9                                                             |
| 1,500                  | 22.2 to 29.2                                             | 18.2 to 25.2                                                             |
| 1,600                  | 25.5 to 32.5                                             | 21.5 to 28.5                                                             |
| 1,700                  | 28.8 to 35.8                                             | 24.8 to 31.8                                                             |
| 1,800                  | 32.1 to 39.1                                             | 28.1 to 35.1                                                             |
| 1,900                  | 35.4 to 42.4                                             | 31.4 to 38.4                                                             |
| 2,000                  | 38.7 to 45.7                                             | 34.7 to 41.7                                                             |
| 2,100                  | 42.0 to 49.0                                             | 38.0 to 45.0                                                             |
| 2,200                  | 45.3 to 52.3                                             | 41.3 to 48.3                                                             |
| 2,300                  | 48.6 to 55.6                                             | 44.6 to 51.6                                                             |
| 2,400                  | 51.9 to 58.9                                             | 47.9 to 54.9                                                             |
| 2,500                  | 55.2 to 62.2                                             | 51.2 to 58.2                                                             |

TABLE IV.—1.5% OXYGEN ENRICHMENT

40

| Blast Temperature, °F. | Moisture expected to be required (grains per cubic foot) | Moisture required according to present invention (grains per cubic foot) |
|------------------------|----------------------------------------------------------|--------------------------------------------------------------------------|
| 1,100                  | 4 to 8                                                   | 4 to 8                                                                   |
| 1,200                  | 7.3 to 11.3                                              | 7.3 to 11.3                                                              |
| 1,300                  | 10.6 to 14.6                                             | 10.6 to 14.6                                                             |
| 1,400                  | 13.9 to 17.9                                             | 11.9 to 14.9                                                             |
| 1,500                  | 17.2 to 21.2                                             | 13.2 to 17.2                                                             |
| 1,600                  | 20.5 to 24.5                                             | 16.5 to 20.5                                                             |
| 1,700                  | 23.8 to 27.8                                             | 19.8 to 23.8                                                             |
| 1,800                  | 27.1 to 31.1                                             | 23.1 to 27.1                                                             |
| 1,900                  | 30.4 to 34.4                                             | 26.4 to 30.4                                                             |
| 2,000                  | 33.7 to 37.7                                             | 29.7 to 33.7                                                             |
| 2,100                  | 37.0 to 41.0                                             | 33.0 to 37.0                                                             |
| 2,200                  | 40.3 to 44.3                                             | 36.3 to 41.3                                                             |
| 2,300                  | 43.6 to 47.6                                             | 39.6 to 43.6                                                             |
| 2,400                  | 46.9 to 50.9                                             | 42.9 to 46.9                                                             |
| 2,500                  | 50.2 to 54.2                                             | 46.2 to 50.2                                                             |

45

| Blast Temperature, °F. | Moisture expected to be required (grains per cubic foot) | Moisture required according to present invention (grains per cubic foot) |
|------------------------|----------------------------------------------------------|--------------------------------------------------------------------------|
| 1,100                  | 11 to 19                                                 | 11 to 19                                                                 |
| 1,200                  | 14.3 to 22.3                                             | 14.3 to 22.3                                                             |
| 1,300                  | 17.6 to 25.6                                             | 17.6 to 25.6                                                             |
| 1,400                  | 20.9 to 28.9                                             | 20.9 to 28.9                                                             |
| 1,500                  | 24.2 to 32.2                                             | 20.2 to 28.2                                                             |
| 1,600                  | 27.5 to 35.5                                             | 23.5 to 31.5                                                             |
| 1,700                  | 30.8 to 38.8                                             | 26.8 to 34.8                                                             |
| 1,800                  | 34.1 to 42.1                                             | 30.1 to 38.1                                                             |
| 1,900                  | 37.4 to 45.4                                             | 33.4 to 41.4                                                             |
| 2,000                  | 40.7 to 48.7                                             | 36.7 to 44.7                                                             |
| 2,100                  | 44.0 to 52.0                                             | 40.0 to 48.0                                                             |
| 2,200                  | 47.3 to 55.3                                             | 43.3 to 51.3                                                             |
| 2,300                  | 50.6 to 58.6                                             | 46.6 to 54.6                                                             |
| 2,400                  | 53.9 to 61.9                                             | 49.9 to 57.9                                                             |
| 2,500                  | 57.2 to 65.2                                             | 53.2 to 61.2                                                             |

TABLE V.—2.0% OXYGEN ENRICHMENT

60

| Blast Temperature, °F. | Moisture expected to be required (grains per cubic foot) | Moisture required according to present invention (grains per cubic foot) |
|------------------------|----------------------------------------------------------|--------------------------------------------------------------------------|
| 1,100                  | 5 to 10                                                  | 5 to 10                                                                  |
| 1,200                  | 8.3 to 13.3                                              | 8.3 to 13.3                                                              |
| 1,300                  | 11.6 to 16.6                                             | 11.6 to 16.6                                                             |
| 1,400                  | 14.9 to 19.9                                             | 14.9 to 19.9                                                             |
| 1,500                  | 18.2 to 23.2                                             | 14.2 to 19.2                                                             |
| 1,600                  | 21.5 to 26.5                                             | 17.5 to 22.5                                                             |
| 1,700                  | 24.8 to 29.8                                             | 20.8 to 25.8                                                             |
| 1,800                  | 28.1 to 33.1                                             | 24.1 to 29.1                                                             |
| 1,900                  | 31.4 to 36.4                                             | 27.4 to 32.4                                                             |
| 2,000                  | 34.7 to 39.7                                             | 30.7 to 35.7                                                             |
| 2,100                  | 38.0 to 43.0                                             | 34.0 to 39.0                                                             |
| 2,200                  | 41.3 to 46.3                                             | 37.3 to 42.3                                                             |
| 2,300                  | 44.6 to 49.6                                             | 40.6 to 45.6                                                             |
| 2,400                  | 47.9 to 52.9                                             | 43.9 to 48.9                                                             |
| 2,500                  | 51.2 to 56.2                                             | 47.2 to 52.2                                                             |

65

| Blast Temperature, °F. | Moisture expected to be required (grains per cubic foot) | Moisture required according to present invention (grains per cubic foot) |
|------------------------|----------------------------------------------------------|--------------------------------------------------------------------------|
| 1,100                  | 13 to 22                                                 | 13 to 22                                                                 |
| 1,200                  | 16.3 to 25.3                                             | 16.3 to 25.3                                                             |
| 1,300                  | 19.6 to 28.6                                             | 19.6 to 28.6                                                             |
| 1,400                  | 22.9 to 31.9                                             | 22.9 to 31.9                                                             |
| 1,500                  | 26.2 to 35.2                                             | 22.2 to 31.2                                                             |
| 1,600                  | 29.5 to 38.5                                             | 25.5 to 34.5                                                             |
| 1,700                  | 32.8 to 41.8                                             | 28.8 to 37.8                                                             |
| 1,800                  | 36.1 to 45.1                                             | 34.1 to 41.1                                                             |
| 1,900                  | 39.4 to 48.4                                             | 35.4 to 44.4                                                             |
| 2,000                  | 42.7 to 51.7                                             | 38.7 to 47.7                                                             |
| 2,100                  | 46.0 to 55.0                                             | 42.0 to 51.0                                                             |
| 2,200                  | 49.3 to 58.3                                             | 45.3 to 54.3                                                             |
| 2,300                  | 52.6 to 61.6                                             | 48.6 to 57.6                                                             |
| 2,400                  | 55.9 to 64.9                                             | 51.9 to 60.9                                                             |
| 2,500                  | 59.2 to 68.2                                             | 55.2 to 64.2                                                             |

TABLE IX.—4.0% OXYGEN ENRICHMENT

70

75

TABLE X.—4.5% OXYGEN ENRICHMENT

| Blast Temperature, °F. | Moisture expected to be required (grains per cubic foot) | Moisture required according to present invention (grains per cubic foot) |
|------------------------|----------------------------------------------------------|--------------------------------------------------------------------------|
| 1,100                  | 15 to 25                                                 | 15 to 25                                                                 |
| 1,200                  | 18.3 to 28.3                                             | 18.3 to 28.3                                                             |
| 1,300                  | 21.6 to 31.6                                             | 21.6 to 31.6                                                             |
| 1,400                  | 24.9 to 34.9                                             | 24.9 to 34.9                                                             |
| 1,500                  | 28.2 to 38.2                                             | 24.2 to 34.2                                                             |
| 1,600                  | 31.5 to 41.5                                             | 27.5 to 37.5                                                             |
| 1,700                  | 34.8 to 44.8                                             | 30.8 to 40.8                                                             |
| 1,800                  | 38.1 to 48.1                                             | 34.1 to 44.1                                                             |
| 1,900                  | 41.4 to 51.4                                             | 37.4 to 47.4                                                             |
| 2,000                  | 44.7 to 54.7                                             | 40.7 to 50.7                                                             |
| 2,100                  | 48.0 to 58.0                                             | 44.0 to 54.0                                                             |
| 2,200                  | 51.3 to 61.3                                             | 47.3 to 57.3                                                             |
| 2,300                  | 54.6 to 64.6                                             | 50.6 to 60.6                                                             |
| 2,400                  | 57.9 to 67.9                                             | 53.9 to 63.9                                                             |
| 2,500                  | 61.2 to 71.2                                             | 57.2 to 67.2                                                             |

TABLE XI.—5.0% OXYGEN ENRICHMENT

| Blast Temperature, °F. | Moisture expected to be required (grains per cubic foot) | Moisture required according to present invention (grains per cubic foot) |
|------------------------|----------------------------------------------------------|--------------------------------------------------------------------------|
| 1,100                  | 17 to 28                                                 | 17 to 28                                                                 |
| 1,200                  | 20.3 to 31.3                                             | 20.3 to 31.3                                                             |
| 1,300                  | 23.6 to 34.6                                             | 23.6 to 34.6                                                             |
| 1,400                  | 26.9 to 37.9                                             | 26.9 to 37.9                                                             |
| 1,500                  | 30.2 to 41.2                                             | 26.2 to 37.2                                                             |
| 1,600                  | 33.5 to 44.5                                             | 29.5 to 40.5                                                             |
| 1,700                  | 36.8 to 47.8                                             | 32.8 to 43.8                                                             |
| 1,800                  | 40.1 to 51.1                                             | 36.1 to 47.1                                                             |
| 1,900                  | 43.4 to 54.4                                             | 39.4 to 50.4                                                             |
| 2,000                  | 46.7 to 57.7                                             | 42.7 to 53.7                                                             |
| 2,100                  | 50.0 to 61.0                                             | 46.0 to 57.0                                                             |
| 2,200                  | 53.3 to 64.3                                             | 49.3 to 60.3                                                             |
| 2,300                  | 56.6 to 67.6                                             | 52.6 to 63.6                                                             |
| 2,400                  | 59.9 to 70.9                                             | 55.9 to 66.9                                                             |
| 2,500                  | 63.2 to 74.2                                             | 59.2 to 70.2                                                             |

It was believed in the past that the quantity of moisture required in blast gas for maintaining a smoothly operating furnace is a function of the percentage of oxygen enrichment and of the blast gas temperature and that the total moisture required is, for all practical purposes, a summation of the moisture necessary for the oxygen enrichment and the moisture necessary for the blast gas temperature. Tables II through XI, under the heading "Moisture expected to be required," disclose ranges of moisture required for different percentages of oxygen enrichment and blast gas temperatures according to this prior understanding of blast furnace operation.

It has been determined from observing actual furnace operations that unexpected advantages are realized by utilizing blast gas heated to a temperature above a critical range. In particular it has been discovered that blast furnaces blown with blast gas heated to temperatures below 1400° F. require a moisture content that falls within the expected ranges, while with blast gas heated to temperatures above about 1400° F.—1500° F. the quantity of moisture required to maintain a smooth operating furnace is substantially less than the minimum moisture that would be expected to be required according to the prior understanding of blast furnace operations.

In Table XII, Examples A, B, C, D, and E are a tabulation of data obtained when operating identical furnaces having a hearth diameter of 28 feet and a height of 108 feet without oxygen enrichment. Examples F through N are a tabulation of data obtained when operating identical furnaces having a hearth diameter of 25 feet, 6 inches, a height of 100 feet and a working volume stock line to center line of tuyeres of 37,872 cubic feet with 5 oxygen enrichment. The data given are averages of values obtained during the period of operation indicated.

TABLE XII

|                                   | Example A | Example B | Example C | Example D | Example E | Example F | Example G |
|-----------------------------------|-----------|-----------|-----------|-----------|-----------|-----------|-----------|
| Iron Prod., Net Tons Per Day      | 1,499     | 1,958     | 2,236     | 1,963     | 2,301     | 1,501     | 1,613     |
| Iron Prod., Net Tons Per Day S.F. | 1,499     | 1,870     | 2,122     | 1,993     | 2,181     | 1,489     | 1,606     |
| Coke Rate, Lbs. Per Net Ton S.F.  | 1,602     | 1,250     | 1,270     | 1,341     | 1,270     | 1,660     | 1,639     |
| Oxygen Enrichment                 |           |           |           |           |           | 1.65      | 2.98      |
| Wind Blown, c.f.m.                | 78,460    | 92,149    | 97,169    | 105,521   | 101,085   | 75,100    | 74,900    |
| Equivalent Wind, c.f.m.           |           |           |           |           |           | 81,000    | 85,600    |
| Moisture, Grains Per Cu. Ft.      | 11.8      | 17.3      | 18.6      | 14        | 17.2      | 10.70     | 15.88     |
| Sinter, percent                   | 31.6      | 58.9      | 61.4      | 59.9      | 52.2      | 16.1      | 24.9      |
| Lime in Sinter, percent           |           |           |           |           |           | 8         | 8         |
| Oversize, percent                 | 6.9       | 13.8      | 38.0      | 33.2      | 39.4      | 10.4      | 11.1      |
| Fe in Burden, percent             | 52        | 54        | 54        | 53        | 54        | 54.38     | 54.74     |
| Blast Temperature, °F.            | 1,277     | 1,602     | 1,641     | 1,654     | 1,673     | 1,260     | 1,285     |
| Top Temperature, °F.              | 271       | 304       | 301       | 264       | 278       | 305       | 295       |
| Stone Rate, Lbs. Per Net Ton S.F. | 553       | 442       | 337       | 599       | 539       | 715       | 667       |
| Dust Rate, Lbs. Per Net Ton S.F.  | 214       | 146       | 261       | 128       | 182       | 190       | 193       |
| Burden, Lbs. Per Charge           | 28,626    | 76,493    | 80,162    | 75,033    | 78,072    | 25,703    | 27,093    |
| Charges Per Day                   | 188       | 92        | 95        | 95        | 103       | 206.5     | 211.9     |
| Delays, Minutes Per Day           | 54        | 110       | 44        | 91        | 38        | 26.3      | 29.5      |
| Days Operated                     | 31        | 31        | 29        | 30        | 31        | 31        | 31        |
| Slag Volume, Lbs. Per Net Ton     |           |           |           |           |           | 848       | 846       |
| CO/CO <sub>2</sub> Ratio          |           |           |           |           |           | 1.83      | 1.76      |
| Iron Prod., Net Tons Per Day      | 1,596     | 1,582     | 1,820     | 1,601     | 1,685     | 1,720     | 1,822     |
| Iron Prod., Net Tons Per Day S.F. | 1,596     | 1,582     | 1,812     | 1,597     | 1,685     | 1,720     | 1,822     |
| Coke Rate, Lbs. Per Net Ton S.F.  | 1,574     | 1,642     | 1,342     | 1,652     | 1,619     | 1,591     | 1,505     |
| Oxygen Enrichment                 | 3.03      | 3.54      | 1.49      | 3.01      | 4.0       | 4.00      | 4.0       |
| Wind Blown, c.f.m.                | 72,800    | 73,000    | 75,200    | 73,000    | 72,900    | 72,900    | 72,900    |
| Equivalent Wind, c.f.m.           | 83,300    | 85,300    | 80,500    | 83,500    | 86,900    | 86,900    | 86,900    |
| Moisture, Grains Per Cu. Ft.      | 16.82     | 21.37     | 11.92     | 20.01     | 23.88     | 23.96     | 24.15     |
| Sinter, percent                   | 36.3      | 36.6      | 66.6      | 24.6      | 37.5      | 40.4      | 50.0      |
| Lime in Sinter, percent           | 8.10      | 8         | 8         | 8         | 8         | 8         | 8         |
| Oversize, percent                 | 12.8      | 12.8      | 19.9      | 10.8      | 12.7      | 12.7      | 12.7      |
| Fe in Burden, percent             | 54.58     | 54.60     | 56.08     | 54.19     | 54.65     | 54.84     | 55.34     |
| Blast Temperature, °F.            | 1,305     | 1,375     | 1,425     | 1,540     | 1,565     | 1,570     | 1,680     |
| Top Temperature, °F.              | 265       | 260       | 305       | 260       | 235       | 240       | 261       |
| Stone Rate, Lbs. Per Net Ton S.F. | 672       | 742       | 387       | 778       | 766       | 733       | 643       |
| Dust Rate, Lbs. Per Net Ton S.F.  | 127       | 112       | 104       | 139       | 111       | 104       | 84        |
| Burden, Lbs. Per Charge           | 27,899    | 27,423    | 44,612    | 27,250    | 27,166    | 27,381    | 28,000    |
| Charges Per Day                   | 196.5     | 202.2     | 134.7     | 203.5     | 216.8     | 216.2     | 214.3     |
| Delays, Minutes Per Day           | 27.7      | 27.8      | 17.5      | 30.3      | 28.7      | 28.4      | 27.5      |
| Days Operated                     | 31        | 30        | 30        | 31        | 23        | 31        | 8         |
| Slag Volume, Lbs. Per Net Ton     | 900       | 939       | 762       | 920       | 950       | 933       | 872       |
| CO/CO <sub>2</sub> Ratio          | 1.80      | 1.83      |           | 1.76      | 1.72      | 1.72      | 1.71      |

TABLE XIII

|           | Blast Temperature, ° F. | Enriched Oxygen, Percent | Actual Moisture (grains per cubic foot) | Moisture Expected (grains per cubic foot) | Moisture Saving |
|-----------|-------------------------|--------------------------|-----------------------------------------|-------------------------------------------|-----------------|
| Example A | 1,277                   | 0                        | 11.8                                    | 11.8                                      | 0               |
| Example B | 1,602                   | 0                        | 17.3                                    | 22.6                                      | 5.3             |
| Example C | 1,641                   | 0                        | 18.6                                    | 23.9                                      | 5.3             |
| Example D | 1,654                   | 0                        | 14.0                                    | 24.4                                      | 10.0            |
| Example E | 1,673                   | 0                        | 17.2                                    | 25.0                                      | 7.8             |
| Example F | 1,260                   | 1.65                     | 10.7                                    | 9.3-13.3                                  | 0               |
| Example G | 1,285                   | 2.03                     | 15.88                                   | 15.13-22.13                               | 0               |
| Example H | 1,305                   | 3.03                     | 16.82                                   | 15.6-22.6                                 | 0               |
| Example I | 1,375                   | 3.54                     | 21.37                                   | 20.1-28.1                                 | 0               |
| Example J | 1,425                   | 1.49                     | 11.92                                   | 14.7-18.4                                 | 2.8             |
| Example K | 1,540                   | 3.01                     | 20.01                                   | 25.55-33.53                               | 5.52            |
| Example L | 1,565                   | 4.0                      | 23.88                                   | 28.35-37.35                               | 4.48            |
| Example M | 1,570                   | 4.0                      | 23.93                                   | 28.53-37.53                               | 4.57            |
| Example N | 1,580                   | 4.0                      | 24.15                                   | 28.86-37.86                               | 4.71            |

Table XIII is a comparison of moisture content of the blast gas in Examples A through N with the moisture content that would be expected to be required according to Table I for oxygen enrichment and in accordance with general rule of adding 1 grain of moisture for each 30° F. increase in blast gas temperature.

From Table XIII, it is seen that with blast gas temperatures at and below 1375° F. the total moisture actually used in the blast gas in order to maintain a smoothly operating furnace falls roughly within the range of "Moisture expected to be required," while with blast gas temperatures of about 1400° to 1500° F., and above, the moisture actually needed for maintaining a smoothly operating furnace is about four grains or more of moisture per cubic foot of blast gas less than the minimum moisture content expected to be required. Thus, according to the principles of the present invention by blowing blast gas heated to a temperature above 1400° F. and/or enriched with oxygen it is possible to reduce the quantity of moisture in the blast gas by at least four grains per cubic foot of blast gas as compared to the total moisture believed to be necessary. A reduction of four grains of moisture in the blast gas blown to the furnace makes it possible to increase the blast gas temperature by at least 120° F. without additional moisture, as a result the coke consumed per ton of iron produced decreases by the order of 50 to 60 pounds with a corresponding increase in pig iron production. From a comparison of Examples I, J, and K, for the particular blast furnace producing these operational examples, it appears that the critical blast gas temperatures above which the unexpected saving in required moisture is obtained is probably around 1425° F. to 1450° F. However, since blast furnace performance depends upon physical characteristics of the blast furnace and upon variable factors including composition of the burden and physical characteristics of constituents of the burden it is believed the critical temperature for average blast furnace installations falls within the range of about 1400° F. to 1500° F., that is, with blast gas heated to a temperature above about 1400° F. to 1500° F. unexpected savings in required moisture can be realized.

While it is not known precisely why the blowing to a blast furnace of blast gas heated to temperature above about 1400° F. to 1500° F. makes it possible to reduce the moisture required in order to obtain a smoothly operating furnace, it is believed that blast gas temperatures above the critical temperature have some effect upon the combustion zones in front of the tuyeres to reduce the size of the core of substantially solid material in the region of the center of the hearth thus permitting combustion gases to flow more easily upwardly into the stack. It is also possible, but not known as a matter of fact, that the use of oxygen enrichment, which in-

creases the oxygen contact per cubic foot of blast gas while actually decreasing the volume of the blast gas, may have some effect to compensate for the disadvantages resulting from expansion of blast gas with increasing temperature when the blast gas temperature is above the critical temperature of about 1400° F. to 1500° F. Although it cannot be said definitely why the combination of oxygen enrichment and elevated blast gas temperatures above about 1400° F. to 1500° F. results in a reduction in the moisture required in order to obtain a smoothly operating furnace, observations of furnaces in actual operation demonstrate that the unexpected results are obtained.

Tables II through XI include the range of moisture required according to the principles of the present invention for various oxygen enrichment percentages at blast gas temperatures. It will be noted that with blast gas temperatures below 1400° F., the moisture required according to the present invention is similar to the moisture expected to be required, while at blast gas temperatures above 1500° F. the range of moisture required according to the present invention is about four grains per cubic foot less than the moisture expected to be required for similar percentages of oxygen enrichment and blast gas temperatures. Although the examples in Table XII show moisture savings greater than four grains per cubic foot of blast gas can be obtained with some furnaces at high blast gas temperatures and although moisture savings should increase with increasing blast gas temperatures, for the sake of clarity, the ranges of required moisture according to the present invention as set forth in Tables II through XI are based on minimum savings of four grains of moisture per cubic foot of blast gas.

Blast furnaces in existence today are generally capable of operation with blast gas temperatures as high as about 2000° F. providing sufficient stove capacity is available. For operation with blast gas temperatures above 2000° F., it will be necessary to utilize high temperature materials in the construction of certain components of the furnace. Although operation with blast gas temperatures above 2000° F. is planned and high temperature materials necessary for such operation are either in existence or under development, the practical range of blast gas temperatures according to the present invention is from about 1400° F. to 1500° F. and up to about 2000° F. Inasmuch as the quantity of moisture saved by practicing the present invention is believed to increase with increasing blast gas temperatures, and since more efficient overall operation will be obtained when it is possible to operate blast furnaces with higher blast gas temperatures, the operation range of blast gas temperatures extends also from about 2000° F. to 2500° F.

TABLE XIV.—5% TO 10% OXYGEN ENRICHMENT

| Blast Temperature, ° F. | Moisture expected to be required (grains per cubic foot) | Moisture required according to present invention (grains per cubic foot) |
|-------------------------|----------------------------------------------------------|--------------------------------------------------------------------------|
| 1,100                   | 17 to 40                                                 | 17 to 40                                                                 |
| 1,200                   | 20.3 to 43.3                                             | 20.3 to 43.3                                                             |
| 1,300                   | 23.6 to 46.6                                             | 23.6 to 46.6                                                             |
| 1,400                   | 26.9 to 49.9                                             | 26.9 to 49.9                                                             |
| 1,500                   | 30.2 to 53.2                                             | 26.2 to 49.2                                                             |
| 1,600                   | 33.5 to 56.5                                             | 29.5 to 52.5                                                             |
| 1,700                   | 36.8 to 59.8                                             | 32.8 to 55.8                                                             |
| 1,800                   | 40.1 to 63.1                                             | 36.1 to 59.1                                                             |
| 1,900                   | 43.4 to 66.4                                             | 39.4 to 62.4                                                             |
| 2,000                   | 46.7 to 69.7                                             | 42.7 to 65.7                                                             |
| 2,100                   | 50.0 to 73.0                                             | 46.0 to 69.0                                                             |
| 2,200                   | 53.3 to 76.3                                             | 49.3 to 72.3                                                             |
| 2,300                   | 56.6 to 79.6                                             | 52.6 to 75.6                                                             |
| 2,400                   | 59.9 to 82.9                                             | 55.9 to 78.9                                                             |
| 2,500                   | 63.2 to 86.2                                             | 59.2 to 82.2                                                             |

Table XV is a composite of data on moisture required in accordance with the invention taken from earlier Tables II, III V, VII, IX, XI, and XIV. It is to be noted that values for any moisture requirements at intermediate value of temperature and percentage oxygen enrichment may be obtained by interpolation from Table XV.

Table XVI illustrates the increase in furnace efficiency obtained when blow with oxygen enriched blast gas heated to a temperature above about 1400° F. to 1500° F. In this table, various blast gas temperatures are indicated with corresponding percentages of oxygen enrichment together with the quantity of moisture required in order to maintain a smoothly operating furnace. The quantity of carbon consumed is based on blast gas of 100,000 cubic feet of blast gas and the relative driving rate is calculated utilizing as a base 1330 pounds of carbon consumed with blast gas at a temperature of 1100° F.

TABLE XV.—COMPOSITE TABLE; MOISTURE REQUIRED ACCORDING TO PRESENT INVENTION  
[Percent oxygen enrichment]

| Blast Temperature, ° F. | 0            | 1            | 2            | 3            | 4            | 5            | 5 to 10%     |
|-------------------------|--------------|--------------|--------------|--------------|--------------|--------------|--------------|
| 1,400                   | 8.4 to 9.4   |              |              |              |              |              |              |
| 1,500                   | 11.7 to 12.7 | 12.2 to 16.2 | 14.2 to 19.2 | 18.2 to 25.2 | 22.2 to 31.2 | 26.2 to 37.2 | 26.2 to 49.2 |
| 1,600                   | 15.0 to 16.0 | 15.5 to 19.5 | 17.5 to 22.5 | 21.5 to 28.5 | 25.5 to 34.5 | 29.5 to 40.5 | 29.5 to 52.5 |
| 1,700                   | 18.3 to 19.3 | 18.8 to 22.8 | 20.8 to 25.8 | 24.8 to 31.8 | 28.8 to 37.8 | 32.8 to 43.8 | 32.8 to 55.8 |
| 1,800                   | 21.6 to 22.6 | 22.1 to 26.1 | 24.1 to 29.1 | 28.1 to 35.1 | 34.1 to 41.1 | 36.1 to 47.1 | 36.1 to 59.1 |
| 1,900                   | 24.9 to 25.9 | 25.4 to 29.4 | 27.4 to 32.4 | 31.4 to 38.4 | 35.4 to 44.4 | 39.4 to 50.4 | 39.4 to 62.4 |
| 2,000                   | 28.2 to 29.2 | 28.7 to 32.7 | 30.7 to 35.7 | 34.7 to 41.7 | 38.7 to 47.7 | 42.7 to 53.7 | 42.7 to 65.7 |
| 2,100                   | 31.5 to 32.5 | 32.0 to 36.0 | 34.0 to 39.0 | 38.0 to 45.0 | 42.0 to 51.0 | 46.0 to 57.0 | 46.0 to 69.0 |
| 2,200                   | 34.8 to 35.8 | 35.3 to 39.3 | 37.3 to 42.3 | 41.3 to 48.3 | 45.3 to 54.3 | 49.3 to 60.3 | 49.3 to 72.3 |
| 2,300                   | 38.1 to 39.1 | 38.6 to 42.6 | 40.6 to 45.6 | 44.6 to 51.6 | 48.6 to 57.6 | 52.6 to 63.6 | 52.6 to 75.6 |
| 2,400                   | 41.4 to 42.4 | 41.9 to 45.9 | 43.9 to 48.9 | 47.9 to 54.9 | 51.9 to 60.9 | 55.9 to 66.9 | 55.9 to 78.9 |
| 2,500                   | 44.7 to 45.7 | 45.2 to 49.2 | 47.2 to 52.2 | 51.2 to 58.2 | 55.2 to 64.2 | 59.2 to 70.2 | 59.2 to 82.2 |

TABLE XVI

| Blast Temperature, ° F. | Oxygen Enrichment, percent | Moisture (grains per cubic foot) | Oxygen in Blast, percent | Moisture in Blast, percent | Pounds of Carbon Consumed | Relative Driving Rate |
|-------------------------|----------------------------|----------------------------------|--------------------------|----------------------------|---------------------------|-----------------------|
| 1,200                   | 1                          | 7.0                              | 21.54                    | 2.1                        | 1,431                     | 1.075                 |
| 1,500                   | 1                          | 17.0                             | 20.90                    | 5.1                        | 1,486                     | 1.115                 |
| 1,800                   | 1                          | 27.5                             | 20.20                    | 8.25                       | 1,542                     | 1.160                 |
| 2,100                   | 1                          | 36.0                             | 19.7                     | 10.8                       | 1,590                     | 1.195                 |
| 2,400                   | 1                          | 45.0                             | 19.2                     | 13.5                       | 1,642                     | 1.235                 |
| 1,200                   | 5                          | 20.0                             | 24.44                    | 6.0                        | 1,740                     | 1.310                 |
| 1,500                   | 5                          | 30.0                             | 23.66                    | 9.0                        | 1,785                     | 1.340                 |
| 1,800                   | 5                          | 40.0                             | 23.1                     | 12.0                       | 1,845                     | 1.383                 |
| 2,100                   | 5                          | 50.0                             | 22.5                     | 15.0                       | 1,900                     | 1.43                  |
| 2,400                   | 5                          | 60.0                             | 21.9                     | 18.0                       | 1,960                     | 1.47                  |
| 1,200                   | 10                         | 33.0                             | 27.93                    | 9.9                        | 2,084                     | 1.570                 |
| 1,500                   | 10                         | 43.0                             | 27.00                    | 12.9                       | 2,119                     | 1.595                 |
| 1,800                   | 10                         | 53.0                             | 26.7                     | 15.9                       | 2,155                     | 1.620                 |
| 2,100                   | 10                         | 63.0                             | 26.1                     | 18.9                       | 2,250                     | 1.69                  |
| 2,400                   | 10                         | 73.0                             | 25.4                     | 21.9                       | 2,304                     | 1.73                  |

Although Tables II through XI show the expected moisture required and the moisture required according to the present invention for percentages of oxygen enrichment from 1 to 5, which range of oxygen enrichment percentages may be economically obtained with presently available equipment, it is known that greater increases in iron production may be obtained by increasing the percentage of oxygen enrichment up to about 10%, for example, and it is expected that blast furnaces will be operated in the future with such high percentages of oxygen enrichment. Table XIV discloses calculated ranges of moisture that would be expected to be required and that would be required according to the principles of the present invention for blast gas having an oxygen enrichment between 5% and 10% at temperatures from 1100° F. to 2500° F. Although this table shows that operation in accordance with the principles of the present invention, that is, at blast gas temperatures about 1400° F. to 1500° F., makes it possible to obtain a reduction in required moisture of four grains per cubic foot of blast gas, it is to be expected, as mentioned above, that the actual moisture saving will be greater especially at higher blast gas temperatures.

without oxygen enrichment and without moisture addition.

It is seen from Table XIV that furnace efficiency increases as the percentage of oxygen enrichment increases. However, at the present time it is not economical to operate furnaces with oxygen enrichment of the order of 10%, for example, in view of the present lack of facilities of oxygen producing equipment of the necessary capacity. Accordingly, for practicing the present invention the practical range of oxygen enrichment is from about 1% to 5%, while the preferred range is from about 5% to 10%.

The teachings of the present invention are applicable, with or without oxygen enrichment, no matter how moisture or its control equivalent is added to the furnace. For example, it has been discovered that the high blast temperatures taught by the invention permit, in fact, actually are required for, auxiliary fuel additions to the blast furnace. As will be described in more detail in subsequent paragraphs, these auxiliary fuels have many of the same effects thermodynamically as aqueous additions and for many purposes can be considered control equivalents. The teachings of the invention include meth-

ods for taking full advantage of such auxiliary fuel additions so that, in combination with reduced moisture additions, a smooth operating furnace is obtained, the coke-rate reduced, and the production rate increased at substantial economic savings over conventional practice.

By auxiliary fuel additions is meant fuel introduced through the tuyeres or other than through the top of the furnace. As pointed out earlier, conventionally, limestone, ferrous bearing material, and carbonaceous material such as coke are charged into the top of the furnace. The charge moves down the shaft of the furnace and the coke, constituting the fuel of the mixture, is burned by the incoming blast to melt the iron producing molten pig iron. Auxiliary fuels, on the other hand, are not introduced at the top of the furnace but near the bottom of the furnace, preferably, in accordance with the invention, through the main tuyeres of the furnace and may include fuels such as natural gas, coke oven gas, fuel oil, powdered carbonaceous materials such as coal, char or coke, or the products of combustion of these fuels.

The problems, economic and otherwise, of acquiring and using quality coke in blast furnace operations are well known in the art. The economic supplanting of quality blast furnace coke with auxiliary fuels is a desirable object. By supplying such auxiliary fuels through the sides of the furnace, for example with the blast, the heat supplied through the blast is increased and it would ordinarily be expected that moisture additions should be increased proportionally. However the complex reactions taking place within the furnace present problems of furnace control, solution loss, and economic use of auxiliary fuels which, it has been discovered dictate processes other than expected. In actuality, a furnace being operated at high blast temperatures and reduced moisture additions in accordance with the invention, must have the moisture additions further reduced in order to economically use auxiliary fuel additions. That is, when a blast furnace is operated with blast gas temperature above about 1400-1500° F. and with auxiliary fuel additions, optimum results can only be obtained with aqueous additions less than the reduced additions set forth in Tables II to XI.

In explaining the invention, natural gas will be used as an example of the auxiliary fuel although the invention is not to be limited thereby. When adding natural gas to a blast furnace the following reactions are believed to have significance:

- A.  $\text{CH}_4 + \frac{1}{2}\text{O}_2 \rightarrow \text{CO} + 2\text{H}_2$
- B.  $\text{CH}_4 + 2\text{O}_2 \rightarrow \text{CO}_2 + 2\text{H}_2\text{O}$ 
  - (1)  $\text{CO}_2 + \text{C} \rightleftharpoons 2\text{CO}_2$
  - (2)  $\text{H}_2\text{O} + \text{C} \rightarrow \text{CO} + \text{H}_2$
- C.  $2\text{C} + \text{O}_2 \rightarrow 2\text{CO}$

Consider the situation where natural gas is added prior to the tuyeres, for example burned in the wind prior to the blast furnace stoves. In such case the formula B above is applicable because the natural gas is burned with a surplus of oxygen and it adds heat to the blast plus the products of combustion  $\text{CO}_2$  and  $\text{H}_2\text{O}$ ; moisture or its control equivalent is being added to the furnace when fuel is added in this fashion.  $\text{CO}_2$  has the same thermodynamic effect as  $\text{H}_2\text{O}$  as it requires heat to dissociate (see Formula B(1)). As pointed out earlier it has been discovered that when making auxiliary fuel additions it is necessary to operate the furnace at higher blast temperatures in order to economically take advantage of the auxiliary fuel. When operating at higher blast temperatures the moisture additions are expected to increase and normally would be increased to obtain a smooth operating furnace. Since fuel additions add moisture, or its control equivalent, a surplus of moisture results and the furnace runs cold. However, it has been discovered that a blast furnace operated on moisture additions can be operated with a precise and predetermined reduction in moisture additions to counteract the moisture and carbon dioxide

produced by burning injected fuel. By reducing the amount of moisture additions in an amount equivalent to the endothermic requirements of the products of combustion of injected fuel, it is possible to obtain the full economic benefits of the auxiliary fuel in improved blast furnace operations including reduction of the coke rate in accordance with the exothermic equivalents of the auxiliary fuel and the reducing agents added thereby.

The burning of auxiliary fuel in the blast presents certain problems, however. For one thing, the refractories in the blast furnace stoves and the mains would have to be replaced in order to withstand the high temperatures of the burning auxiliary fuel. With the extremely high temperatures of the blast encountered heat losses are increased before the blast reaches the furnace and yet the products of combustion of the auxiliary fuel would require additional heat once inside the furnace to be dissociated and made available as reducing agents. Therefore, practically speaking, it has been discovered that it is more economically feasible to add the natural gas, or other auxiliary fuel, at the tuyeres.

When adding the natural gas at the tuyeres the reaction set forth in A above can take place within the furnace. That is the auxiliary fuel burns in a shortage of oxygen and  $\text{CO}$  and  $\text{H}_2$ , reducing agents, are formed directly. The question presented is what effect does this reaction have on the endothermic requirements of auxiliary fuel additions. It has been discovered that, disregarding plant heat losses, the endothermic requirements of auxiliary fuel additions are approximately the same whether added at the tuyeres or burned prior to introduction to the furnace. It is believed that the reason for this could be, quite simply, that the same reaction (B above) takes place regardless of where the auxiliary fuel is added. Another explanation behind the endothermic equivalency could be that when reaction A takes place with constant wind the addition of natural gas at the tuyeres reduces the  $\text{O}_2$  available for the C reaction. A reduction in the C reaction reduces the heat available in the furnace, as this reaction is more exothermic than the A reaction since the coke is already heated and inherently produces more heat in combustion. The natural gas, being gaseous, is more readily combustible and to some extent takes the place of coke combustion. Therefore even in the absence of the formation of  $\text{H}_2\text{O}$  and  $\text{CO}_2$ , the introduction of natural gas into the tuyeres produces the same overall effect as adding moisture in spite of the fact that neither  $\text{H}_2\text{O}$  nor  $\text{CO}_2$  may be formed. Therefore whether the auxiliary fuel is burned before entering the furnace or added at the tuyeres a reduction in moisture additions is required in proportion to the products of combustion of auxiliary fuel when a like amount of auxiliary fuel is burned in a surplusage of oxygen. However, the teachings of the invention emphasize the advantages of introducing the auxiliary fuel at the tuyeres, such as the avoidance of plant heat losses.

Examples of blast furnace operations, using moisture additions for furnace control, with and without auxiliary fuel additions, are included in Table XVII to follow. The experimental data included therein are averages of values obtained during the operation periods indicated. The experimental blast furnace employed has a hearth diameter of four feet, a height of approximately 26 feet, and a working volume of approximately 305 cubic feet. Owing to the greater heat losses per unit of production in an experimental furnace of this size, as compared to a commercial furnace, higher blast temperatures are employed and must be converted for commercial furnace application based on established conversion tables recognized in the art as follows:

| Experimental Furnace: | Commercial Furnace, ° F. |
|-----------------------|--------------------------|
| 1,600° F.             | 1,250                    |
| 1,800° F.             | 1,425                    |
| 2,100° F.             | 1,700                    |
| 2,475° F.             | 2,000                    |

|                               | Example 1 | Example 2 | Example 3 | Example 4 |
|-------------------------------|-----------|-----------|-----------|-----------|
| <b>FURNACE PERFORMANCE</b>    |           |           |           |           |
| Iron Prod., Net Tons Per Day  | 18.74     | 18.91     | 20.82     | 18.31     |
| Coke Rate, Lbs. Per Net Ton   | 1,322     | 1,096     | 1,104     | 1,105     |
| Slag Volume, Lbs. Per Net Ton | 985       | 993       | 957       | 1,005     |
| <b>OPERATING CONDITIONS</b>   |           |           |           |           |
| Oxygen Enrichment             |           |           | 20        |           |
| Wind Rate, c.f.m.             | 800       | 800       | 800       | 800       |
| Moisture, Grains Per Cu. Ft.  | 27        | 6.8       | 5.6       | 4         |
| Gas Injec. Rate, c.f.m.       |           | 40        | 40        | 40        |
| Blast Temp., ° F.             | 2,475     | 2,475     | 2,475     | 2,475     |
| Top Temp., ° F.               | 328       | 458       | 349       | 452       |
| <b>HOT METAL DATA</b>         |           |           |           |           |
| Silicon, Percent              | 0.88      | 0.77      | 0.88      | 0.74      |
| Sulfur, Percent               | 0.039     | 0.045     | 0.031     | 0.038     |
| Temperature, ° F.             | 2,515     | 2,490     | 2,525     | 2,499     |
| Number of Casts               | 24        | 12        | 28        | 16        |
| Hours of Operation            | 72        | 122       | 27        | 55        |

It can be seen from the above data that the use of auxiliary fuel and high blast temperatures brings about an increased metal production rate and a decreased coke rate. Additional coke savings are realized from the carbon of the auxiliary fuel which replaces carbon from the burden coke.

An important discovery of the invention is that fuel additions cannot be economically used without increasing the blast temperature. The production rate of a furnace will increase directly with auxiliary fuel additions if the cooling effect of the auxiliary fuel and aqueous additions are compensated for by increased blast temperatures and decreased aqueous additions. In practice, the necessary increase in temperature has amounted to about 120° F. for each percent of auxiliary fuel (natural gas) added. The necessary increase in blast temperature with auxiliary fuels would not be as high as 120° F. with each percent of auxiliary fuel addition if a more exothermic fuel than natural gas, such as powdered coal, were used. Within the practical limits of blast temperatures imposed at most blast furnace sites today the maximum percentage of natural gas which could be effectively used would be around 5 to 6% by volume of the blast. With more exothermic auxiliary fuels the percentage may be increased to 8% or beyond.

As pointed out earlier about one grain of moisture per cubic foot of blast gas is added with each 30° increase in blast gas temperature. For each percent by volume natural gas added blast gas temperature should be increased approximately 120°. From this data it can be seen that, as far as blast furnace control is concerned, one percent of natural gas is approximately equivalent, considering smooth operations, to four grains of moisture. In other words, when making auxiliary fuel additions of natural gas, for each percent of natural gas added to the blast, the aqueous additions should be reduced approximately four grains.

The reduction in aqueous additions is not without limitation, however. A significant discovery, forming part of the invention, is that aqueous additions should not be eliminated entirely. In practice, the furnace cannot be readily controlled by adjusting the rate of auxiliary fuel injections, but excellent control can be obtained by maintaining some aqueous additions to the furnace.

The reasons why the auxiliary fuel is not effective in instantaneous control, even though it serves as an equivalent in many other respects to aqueous addition, are multiple and speculative. Mostly, the explanations hinge on the change in the amount of carbon available in the furnaces with changes in the auxiliary fuel injection rate. Consider a furnace which is hanging and the area beneath a bridge or scaffolding causing the furnace to hang is becoming increasingly hot. Ideally, aqueous additions or the moisture additions effect of adding auxiliary fuel

would serve to cool this area and lengthen the combustion zone in the furnace and thereby reestablish smooth descent of the burden. In general, cooling of the hot zone takes place with either additive. However, due to the presence of carbon in the auxiliary fuel and the tendency of this carbon to combine with O<sub>2</sub> more readily than the carbon in the coke, there is less coke burned. Descent of the burden will be sluggish because of the lowered demand for burden carbon. On the other hand, aqueous additions effect the necessary cooling and charge only O<sub>2</sub> or H<sub>2</sub> into the furnace so that the burden starts to move more readily. Also, maintaining limited aqueous additions to the furnace permits temperature control of the furnace affecting silicon and sulphur content of the melt without adding carbon to the furnace.

In actual practice, the amount of aqueous additions maintained should be sufficient to exercise furnace control. If dehumidifying equipment is not used, aqueous additions of about 7 grains are sufficient to allow for normal variations in the ambient atmospheric humidity and leave a margin for varying the aqueous addition to effect instantaneous control. If dehumidifying equipment is used on the blast, the aqueous additions to the furnace helpful in instantaneous control can be maintained by regulating the humidity of the air used in the blast.

In summary, when using auxiliary fuel, to obtain an increased production from a blast furnace, the blast gas temperature should be increased and the aqueous additions reduced in accordance with the endothermic requirements of the auxiliary fuel. The coke rate should be reduced in accordance with the carbon and reducing agents added by the auxiliary fuel. If oxygen enrichment is used the production rate will be increased since the consumption of the oxygen of the blast by the auxiliary fuel will be reduced and will be available for burning additional coke in the burden and increasing the driving rate.

It is to be expressly understood that various changes and substitutions may be made in the specific embodiments described herein without departing from the spirit of the invention as well understood by those skilled in the art. Therefore, reference will be had to the appended claims for a definition of the limits of the invention.

I claim:

1. Method of operating a blast furnace in which iron bearing material is smelted and in which coke is burned, comprising the steps of forming blast gas including atmospheric air, enriching blast gas with oxygen, adding aqueous fluid to the blast gas, heating the blast gas to a temperature above about 1400° F. to 1500° F., and blowing blast gas into the furnace, the oxygen enrichment being in the range of 1%–10%, and the quantity of aqueous fluid in the blast gas being from about 12.2 to about 82.2 grains of moisture per cubic foot of blast gas, the aqueous fluid in the blast gas increasing from about 12.2 to about 82.2

grains of moisture per cubic foot of blast gas as the oxygen enrichment increases from about 1% to about 10%.

2. Method of operating a blast furnace in which iron bearing material is smelted and in which coke is burned, comprising the steps of forming blast gas including atmospheric air, enriching blast gas with oxygen, adding aqueous fluid to the blast gas, heating the blast gas to a temperature above about 1400° F. to 1500° F., and blowing blast gas into the furnace, the oxygen enrichment being in the range of 1%–5% and the quantity of aqueous fluid in the blast gas being from about 12.2 to about 70.2 grains of moisture per cubic foot of blast gas, the aqueous fluid in the blast gas increasing from about 12.2 to about 70.2 grains of moisture per cubic foot of blast gas as the oxygen enrichment increases from about 1% to about 5%.

3. Method of operating a blast furnace in which iron bearing material is smelted and in which coke is burned, comprising the steps of forming blast gas including atmospheric air, enriching blast gas with oxygen, adding aqueous fluid to the blast gas, heating the blast gas to a temperature above about 1400° F. to about 1500° F., and blowing blast gas into the furnace, the oxygen enrichment being within the range of 5%–10% and the quantity of aqueous fluid in the blast gas being from about 26.2 to about 82.2 grains of moisture per cubic foot of blast gas, the aqueous fluid in the blast gas increasing from about 26.2 to about 82.2 grains of moisture per cubic foot of blast gas as the oxygen enrichment increases from about 5% to about 10%.

4. Method of operating a blast furnace in which iron bearing material is smelted and in which coke is burned, comprising the steps of forming blast gas including atmospheric air, enriching blast gas with oxygen, adding aqueous fluid to the blast gas, heating the blast gas to a temperature above about 1400° F. to 1500° F. and up to 2000° F., and blowing blast gas into the furnace, the oxygen enrichment being in the range of 1% to 10% and the quantity of aqueous fluid in the blast gas being from about 12.2 to about 65.7 grains of moisture per cubic foot of blast gas, the aqueous fluid in the blast gas increasing from about 12.2 to about 65.7 grains of moisture per cubic foot of blast gas as the oxygen enrichment increases from about 1% to about 10%.

5. Method of operating a blast furnace in which iron bearing material is smelted and in which coke is burned, comprising the steps of forming blast gas including atmospheric air, enriching blast gas with oxygen, adding aqueous fluid to the blast gas, heating the blast gas to a temperature above about 1400° F. to 1500° F. and up to about 2000° F., and blowing blast gas into the furnace, the oxygen enrichment in the blast gas being in the range of 1%–5%, and the quantity of aqueous fluid in the blast gas being from about 12.2 to about 53.7 grains of moisture per cubic foot of blast gas, the aqueous fluid in the blast gas increasing from about 12.2 to about 53.7 grains of moisture per cubic foot of blast gas as the oxygen enrichment increases from about 1% to about 5%.

6. Method of operating a blast furnace in which iron bearing material is smelted and in which coke is burned, comprising the steps of forming blast gas including atmospheric air, enriching the blast gas with oxygen, adding aqueous fluid to the blast gas, heating the blast gas to a temperature above about 1400° F. to 1500° F. and up to about 2000° F., and blowing the blast gas into the furnace, the oxygen enrichment being within the range of about 5%–10%, and the quantity of aqueous fluid in the blast gas being from about 26.2 to 65.7 grains of moisture per cubic foot of blast gas, the aqueous fluid in the blast gas increasing from about 26.2 to about 65.7 grains of moisture per cubic foot of blast gas as the oxygen enrichment increases from about 5% to about 10%.

7. Method of operating a blast furnace in which iron

bearing material is smelted and in which coke is burned, comprising the steps of forming blast gas including atmospheric air, enriching blast gas with oxygen, adding aqueous fluid to the blast gas, heating the blast gas to a temperature above about 2000° F. and up to about 2500° F., and blowing blast gas into the furnace, the oxygen enrichment in the blast gas being in the range of 1%–10%, and the quantity of aqueous fluid in the blast gas being from about 28.7 to about 82.2 grains of moisture per cubic foot of blast gas, the aqueous fluid in the blast gas increasing from about 28.7 to about 82.2 grains of moisture per cubic foot of blast gas as the oxygen enrichment increases from about 1% to about 10%.

8. Method of operating a blast furnace in which iron bearing material is smelted and in which coke is burned, comprising the steps of forming blast gas including atmospheric air, enriching blast gas with oxygen, adding aqueous fluid to the blast gas, heating the blast gas to a temperature above about 2000° F. and up to about 2500° F., and blowing blast gas into the furnace, the oxygen enrichment in the blast gas being in the range of 1%–5%, and the quantity of aqueous fluid in the blast gas being from about 28.7 to about 70.2 grains of moisture per cubic foot of blast gas, the aqueous fluid in the blast gas increasing from about 28.7 to about 70.2 grains of moisture per cubic foot of blast gas as the oxygen enrichment increases from about 1% to about 5%.

9. Method of operating a blast furnace in which iron bearing material is smelted and in which coke is burned, comprising the steps of forming blast gas including atmospheric air, enriching blast gas with oxygen, adding aqueous fluid to the blast gas, heating the blast gas to a temperature above about 2000° F. and up to about 2500° F., and blowing blast gas into the furnace, the oxygen enrichment being within the range of 5%–10%, and the quantity of aqueous fluid in the blast gas being from about 42.7 to about 82.2 grains of moisture per cubic foot of blast gas, the aqueous fluid in the blast gas increasing from about 42.7 to about 82.2 grains of moisture per cubic foot of blast gas as the oxygen enrichment increases from about 5% to about 10%.

10. Method of operating a blast furnace in which iron bearing and carbonaceous material are charged into the top of the furnace and a blast gas is introduced into the bottom of the furnace comprising the steps of preheating the blast gas to a temperature above about 1400° F., and adding aqueous fluid to the blast gas in accordance with the temperature of the blast gas, the quantity of aqueous fluid added being about nine grains of aqueous fluid per cubic foot of blast furnace gas at a temperature of about 1400° F. with about three grains of moisture per cubic foot of blast gas required to be added with each 100° F. increase in blast gas temperature above 1400° F.

11. Method of operating a blast furnace in which iron bearing and carbonaceous materials are charged into the top of the furnace and a blast gas is introduced into the bottom of the furnace comprising the steps of preheating the blast gas to temperatures above 1400° F., adding aqueous fluid to the blast gas with about 9 grains of aqueous fluid per cubic foot of blast gas being added at 1400° F., adding auxiliary fuel to the blast gas in the range of about 1% to about 8% by volume of the blast gas, and controlling the blast gas temperature in accordance with the formula, blast gas temperature =  $1400 + (M)33 + (F)120$ ° F., wherein M is equal to the grains of aqueous fluid above 9 grains per cubic foot of blast gas added and F is equal to the percentage of the blast gas by volume auxiliary fuel added to the blast gas.

12. In a process of heating and humidifying the blast for a metallurgical blast furnace, which comprises: blowing cold blast air for the blast of the furnace through a preheating medium therefor and thereby preheating the blast for the furnace, thereafter augmenting the heat of the blast from said medium by burning combustible fuel

with part of the total air of the blast directly in the pre-heated blast, and thereafter delivering the heat augmented hot blast into the hearth in the blast furnace while charged with water vapor to a predetermined constancy of humidity, the improvement comprising the steps of; effecting said augmenting of the heat of the blast by burning a hydrogen containing fuel as the combustible fuel directly in the blast and thereby charging the blast with a substantial part of the water vapor for said predetermined constancy of humidity as a product of said combustion, and adding the remainder of the total amount of vapor to form said predetermined constancy of humidity in the form of aqueous fluid to the blast before the heat of the blast is augmented.

13. A process as claimed in claim 12, and in which the preheating by the aforesaid preheating medium is effected by regenerative heating of the blast by heat previously stored in heat storing material.

14. A method as claimed in claim 12, and in which the amounts of the hydrogen containing gas that is burned as aforesaid, and of the part of the total air of the blast that is burned with the gas, is controlled by, and in accordance with variations in the total amount of cold blast air blown in the first aforesaid blowing step for the blast.

15. Method of operating a blast furnace in which iron bearing material and carbonaceous material are charged into the top of the furnace and blast gas is introduced at the bottom of the furnace, comprising the steps of pre-heating the blast gas to a predetermined temperature, adding auxiliary fuel to the blast gas, and adding aqueous fluid to the blast gas in accordance with the temperature of the blast gas and the endothermic requirements of the auxiliary fuel, the quantity of aqueous fluid being substantially equal to the aqueous fluid required at the predetermined temperature without auxiliary fuel being introduced into the furnace and a quantity of aqueous fluid equivalent to the endothermic requirements of the auxiliary fuel, the quantity of aqueous fluid required to be added to the blast gas at the predetermined temperature being from about 9 grains per cubic foot of blast gas at a temperature of about 1400° F. with about 3 grains of aqueous fluid per cubic foot of blast gas required to be added for each 100° F. increase in blast gas temperature above 1400° F.

16. The method of operating a blast furnace as defined in claim 15 including the step of controlling the quantity of carbonaceous material charged into the top of the blast furnace based on the exothermic equivalent of the auxiliary fuel added to the blast gas.

17. The method of operating a blast furnace as defined in claim 15 in which the auxiliary fuel comprises natural gas added in the range of about 1 percent to about 8 percent by volume of the blast gas.

18. Method of operating a blast furnace in which iron bearing material and carbonaceous material are charged into the top of the furnace and blast gas is introduced through blast furnace tuyeres at the bottom of the furnace comprising the steps of preheating the blast gas to a predetermined temperature, adding aqueous fluid to the blast gas, adding auxiliary fuel at the blast furnace tuyeres, and controlling the aqueous fluid additions to the blast gas in accordance with the temperature of the blast gas and the endothermic requirements of the auxiliary fuel, the quantity of aqueous fluid additions being substantially equal to the aqueous fluid required at the predetermined blast gas temperature offset by equivalent aqueous fluid substantially equal to the endothermic requirements of the added auxiliary fuel, the quantity of aqueous fluid required at the predetermined blast gas temperature being approximately 9 grains per cubic foot of blast gas at a temperature of about 1400° F. with 3 grains of aqueous additions per cubic foot of blast gas being added for each 100° F. increase in blast gas temperature above 1400° F.

19. Method of operating a blast furnace in which iron

bearing material and carbonaceous material are charged into the top of the furnace and blast gas is introduced into the bottom of the furnace comprising the steps of pre-heating the blast gas to a predetermined temperature, adding auxiliary fuel to the blast gas, and adding aqueous fluid to the blast gas in accordance with the temperature of the blast gas and the endothermic requirements of the auxiliary fuel, the quantity of aqueous fluid added to the blast gas being substantially equal to the difference between the quantity of aqueous fluid required to be added to blast gas at the predetermined temperature without auxiliary fuel being introduced into the furnace and a quantity of aqueous fluid equivalent to the endothermic requirements of the auxiliary fuel, the quantity of aqueous fluid required to be added to the blast gas without auxiliary fuel introduced into the furnace varying between about 9 grains of aqueous fluid per cubic foot of blast gas at 1400° F. and about 45 grains of aqueous fluid per cubic foot of blast gas at 2500° F.

20. Method of operating a blast furnace in which iron bearing material and carbonaceous material are charged into the top of the furnace and blast gas is introduced into the bottom of the furnace comprising the steps of pre-heating the blast gas to a predetermined temperature, enriching the blast gas with a predetermined percentage of oxygen, in the range of about 1% to about 10% of the blast gas, adding auxiliary fuel to the blast gas, and adding aqueous fluid to the blast gas in accordance with the temperature of the blast gas, the percent of oxygen enrichment and the endothermic requirements of the auxiliary fuel, the quantity of aqueous fluid added to the blast gas being substantially equal to the difference between the quantity of aqueous fluid required to be added to blast gas at the predetermined temperature and the predetermined percentage of oxygen enrichment without auxiliary fuel introduced into the furnace and the quantity of aqueous fluid equivalent to the endothermic requirements of the auxiliary fuel, the quantity of aqueous fluid required to be added to the blast gas without auxiliary fuel introduced into the furnace varying between about 12 grains of aqueous fluid per cubic foot of blast gas at 1500° F. and 1% oxygen enrichment and about 82 grains of aqueous fluid per cubic foot of blast gas at 2500° F. and about 10% oxygen enrichment.

21. Method of operating a blast furnace in which iron bearing material and carbonaceous material are charged into the top of the furnace and blast gas is introduced into the bottom of the furnace comprising the steps of preheating the blast gas to a predetermined temperature, adding natural gas to the blast gas in the range of about 1 percent to about 6 percent by volume of the blast gas, and adding aqueous fluid to the blast gas in accordance with the temperature of the blast gas and the endothermic requirements of the auxiliary fuel, the quantity of the aqueous fluid additions being equal to the aqueous fluid additions required at the predetermined blast gas temperature offset by equivalent aqueous fluid substantially equal to the endothermic requirements of the added natural gas, the quantity of aqueous fluid additions required by the blast gas temperature being equal to approximately 9 grains per cubic foot of blast gas at a temperature of about 1400° F. with about 3 grains of aqueous additions per cubic foot of blast gas being added for each 100° F. increase in blast temperature above 1400° F. and the equivalent aqueous fluid for the natural gas added being approximately 4 grains of aqueous fluid for each percent by volume of natural gas added to the blast gas.

22. In the operation of a blast furnace in which iron bearing material and carbonaceous material are charged into the top of the furnace and blast gas is introduced at the bottom of the furnace, a method for increasing the production rate of the furnace comprising the steps of adding natural gas to the blast gas in the range of about 1 percent to about 8 percent by volume of the blast gas, and controlling the blast gas temperature in accordance

with the endothermic requirements of the added natural gas, the endothermic requirements being an increase in blast gas temperature of about 120° F. for each percent by volume of natural gas added to the blast gas.

23. Method of operating a blast furnace in which iron bearing material and carbonaceous material are charged into the top of the furnace and a blast gas is introduced at the bottom of the furnace, comprising the steps of pre-heating the blast gas to a predetermined temperature, introducing material into the bottom of the furnace as auxiliary fuel, and adding aqueous fluid to the blast gas in accordance with the temperature of the blast gas and the endothermic requirements of the introduced material, the quantity of aqueous fluid added to the blast gas being substantially equal to the difference between the quantity of aqueous fluid required to be added to the blast gas at the predetermined temperature without auxiliary fuel being introduced into the furnace and a quantity of aqueous fluid equivalent to the endothermic requirements of the introduced material, the predetermined temperature of the blast gas being from about 1400° F. and up to about 2500° F. and the quantity of aqueous fluid required to be added to the blast gas at the predetermined temperature being from about 9 grains of moisture up to about 45 grains of moisture per cubic foot of blast gas, and the quantity of aqueous fluid equivalent to the endothermic requirements of the introduced material being approximately 4 grains of aqueous fluid per cubic foot of blast gas per endothermic requirement N, the endothermic requirement N being equal to the endothermic requirement of a quantity of natural gas equal to 1% of the blast gas.

5

10

15

20

25

30

## References Cited by the Examiner

## UNITED STATES PATENTS

|           |         |               |         |
|-----------|---------|---------------|---------|
| 1,510,271 | 9/1924  | Gottschalk    | 75—41   |
| 2,219,046 | 10/1940 | Koller et al. | 75—42   |
| 2,715,575 | 8/1955  | Coutant       | 75—41   |
| 2,719,083 | 9/1955  | Pomykala      | 75—42   |
| 2,729,555 | 1/1956  | Shipley       | 75—41   |
| 2,735,758 | 2/1956  | Strassburger  | 75—41   |
| 2,778,018 | 1/1957  | Strassburger  | 75—41 X |

## OTHER REFERENCES

Blast Furnace Proceedings, 1958, vol. 17, pages 4—39.  
Iron Age, vol. 184, July 16, 1959, pages 104 and 105 relied on.

Journal of Metals, January 1961, pages 25—30 (also Blast Furnace Proceeding, vol. 19, 1960, pages 238—278).

Metal Progress, August 1949 (pp. 234 and 236 relied on).

Steel, vol. 139, No. 22, Nov. 26, 1956, pages 98, 101, 104, 107, and 110 relied on.

Sweetser, Blast Furnace Practice, 1st Edition, 1938, McGraw-Hill Book Co., Inc., New York (page 253 relied on).

DAVID L. RECK, Primary Examiner.

RAY K. WINDHAM, ROGER L. CAMPBELL,  
Examiners.